

United States Patent [19]  
Yarrington

[11] 3,919,000  
[45] Nov. 11, 1975

- [54] PREANNEAL RINSE PROCESS FOR  
INHIBITING RUST ON STEEL STRIP  
[75] Inventor: Robert Warren Yarrington, Ambler,  
Pa.  
[73] Assignee: Pennwalt Corporation, Philadelphia,  
Pa.  
[22] Filed: June 15, 1973  
[21] Appl. No.: 370,497

- [52] U.S. Cl. .... 148/14  
[51] Int. Cl.<sup>2</sup> .... C21D 1/00  
[58] Field of Search .... 148/4, 6.14, 13.1, 14,  
148/15, 18, 31.5, 20.6, 27; 117/49, 127;  
134/2, 19

[56] References Cited  
UNITED STATES PATENTS

1,260,740 3/1918 Allen ..... 148/6.14 R

3,039,902 6/1962 Miller ..... 148/14 X  
3,052,575 9/1962 Crane ..... 148/6.14 R  
3,257,159 6/1966 Zimmermann ..... 148/6.14 R X  
3,526,552 9/1970 Church et al. .... 148/14

FOREIGN PATENTS OR APPLICATIONS  
1,180,951 2/1970 United Kingdom ..... 148/6.14

Primary Examiner—C. Lovell  
Attorney, Agent, or Firm—Robert G. Danehower

[57] ABSTRACT

Cold rolled steel strip is treated, prior to annealing, with a dilute aqueous rinse solution containing soluble calcium salt or a soluble ferricyanide or ferrocyanide salt or a mixture of soluble calcium salt with sodium nitrite or soluble ferricyanide or soluble ferrocyanide. The residues of said rinses inhibit rust formation on the annealed strip during storage and transit.

5 Claims, No Drawings

**PREANNEAL RINSE PROCESS FOR INHIBITING  
RUST ON STEEL STRIP**

This invention relates to a method of increasing the oxidation (i.e., rust) resistance of ferrous strip, and more particularly concerns the rinse treatment of cold-rolled steel strip, prior to annealing thereof, with a soluble calcium salt or a soluble ferricyanide or ferrocyanide salt or a mixture of the calcium salt with sodium nitrite or the soluble ferricyanide or ferrocyanide, in dilute aqueous solution, to leave a thin layer of the residue from such rinse solution on the strip during annealing and subsequent storage and transit. The rust formation problem with steel strip dealt with by this invention is to be distinguished from the problem of preventing defects in electrolytically coated tinplate (i.e., preventing staining or dewetting of tin-coated surface) in which the steel strip is treated with a dilute aqueous rinse of a material that remains on the strip during batch annealing and is capable of reacting with carbonaceous material thereon during the batch annealing cycle. (Brown et al., U.S. Pat. No. 3,632,487, and a similar treatment for chromium and chromium oxide coated strip, Brown et al. application Ser. No. 231,747, filed Mar. 3, 1972, now U.S. Pat. No. 3,756,926.

Cold-rolled, annealed, steel strip is subject to rusting caused by oxidation of the ferrous metal, particularly where processing water used in the mill has a high content of dissolved chlorides and/or sulfates. The rust formation, which is more pronounced when the coiled strip is in humid environment, reduces the value of the strip for further processing and is often severe enough so that the strip must be scrapped. Shoemaker, in U.S. Pat. No. 3,668,021, offered one solution to the rust problem by disclosing the application of an aqueous suspension (dispersion) of calcium hydroxide to the strip prior to annealing. The disadvantages of this method stem from the water-insolubility of calcium hydroxide. For example, it is necessary to continuously agitate the slurry to provide a uniform dispersion of the suspended solids. In addition, the application of insoluble solids tends to give non-uniform coatings of the rust inhibiting substance which could result in localized pinpoint rusting. Another difficulty is that the residue left from treatment with an insoluble compound can be deposited on the temper rolls in the subsequent processing of the strip.

In accordance with the present invention, the cold-rolled steel strip is treated with an aqueous dilute rinse solution containing an effective rust-inhibiting amount of calcium ion or ferricyanide ion or ferrocyanide ion, or mixture of calcium ion with sodium nitrite or ferricyanide or ferrocyanide ion. (Sodium nitrite has previously been used as a rust inhibitor for ferrous metals, but not for the purpose or in the specific utility embodied herein, and not in combination with a soluble calcium salt component.) The components of the rinse solution of this invention are water-soluble materials, which property provides uniform coatings, simplifies the handling techniques and equipment requirements, and reduces the opportunities for residues to interfere with the temper rolling operation. The soluble calcium salt operable herein has a solubility in water of at least 1.88 g/liter of  $\text{Ca}^{++}$  ion, and preferably at least about 3.76 g/liter of  $\text{Ca}^{++}$  ion (at 70°F.). Representative of such salts are, for example,

calcium acetate

calcium benzoate  
calcium butyrate  
calcium chromate  
calcium ferrocyanide  
calcium ferricyanide  
calcium formate  
calcium fumarate  
calcium d-gluconate  
calcium glycerophosphate  
calcium isobutyrate  
calcium iodide  
calcium lactate  
calcium  $\alpha$ -methylbutyrate  
calcium nitrate  
calcium nitrite  
calcium propionate  
calcium salicylate  
calcium dithionate  
calcium maleate  
calcium valerate

Various salts of calcium whose anions are promoters of corrosion, e.g., calcium sulfate and calcium chloride, are to be avoided, as well as those likely to stain steel during annealing, such as calcium permanganate. Calcium chromate, mentioned above, can be used except where the steel strip is ultimately to be coated with tin because chromate interferes with the tin-plating process.

The soluble ferrocyanide or ferricyanide salts operable herein have a solubility in water of at least 0.94 g/liter of  $\text{Fe}(\text{CN})_6$  moiety and preferably about 1.88 g/liter of ferricyanide or ferrocyanide. Representative of such salts are, for example,

ammonium ferricyanide  
ammonium ferrocyanide  
calcium ferricyanide  
calcium ferrocyanide  
magnesium ferrocyanide  
potassium ferricyanide  
potassium ferrocyanide  
sodium ferricyanide  
sodium ferrocyanide  
strontium ferrocyanide

Before carrying out the process of this invention, it is expedient to subject the cold rolled steel strip to a conventional electrocleaning and rinsing operation, accomplished with a hot aqueous alkaline silicate solution, followed by rinsing and scrubbing. It has been observed that the process of this invention appears to provide a synergistic improvement in subsequent corrosion resistance when used in conjunction with prior electrolytic cleaning with silicates in caustic aqueous solution. The use of alkali silicate solutions for cleaning steel strip (e.g., sodium orthosilicate or sodium metasilicate) is well known and is described, for example, in the articles by L. J. Brown and J. E. Lippy, Jr. in *Plating*, February, 1966, "Silicates as Cleaners in the Production of Tinplate" and II. "Influence of Batch Anneal", October, 1971; and the text by W. E. Hoare et al., *The Technology of Tinplate*, St. Martin's Press, 1965.

Following the foregoing cleaning operation, the strip is contacted with the rust-inhibiting rinse solution embodied herein, either by immersion or by spray application, conveniently at ambient temperature, although rinse temperatures ranging from about 50° to about 200°F. may be employed, temperature of the rinse not being a critical factor. Said dilute aqueous rinse solution, containing in admixture the dissolved calcium salt

or ferricyanide or ferrocyanide, or mixture of calcium ion with the nitrite, ferricyanide or ferrocyanide, above mentioned, will usually have said components present in amounts providing from about 0.25 to 3 ounces of calcium ion per gallon of solution, and from about 0.13 to 3 ounces per gallon of sodium nitrite, or ferricyanide or ferrocyanide ion, when present. Preferred concentrations range from 0.5 to 1.5 oz./gallon of calcium ion and from 0.26 to 1.5 oz./gallon of the additional nitrite or ferrocyanide or ferricyanide ion.

After the brief immersion in or spraying with said rinse solution, the steel strip is permitted to air-dry, either at ambient temperatures or at elevated temperatures, e.g., up to about 300°F., thus depositing a thin uniform film of the rinse solution residues thereon. The treated steel strip is subsequently annealed, using either conventional continuous annealing or batch annealing techniques. In continuous annealing the treated strip is passed through an annealing oven at such a rate to provide an annealing period of approximately 20 seconds at a temperature of about 1200° to 1220°F., followed by a controlled cooling cycle, in a protective gas atmosphere, e.g., consisting of 5 percent hydrogen and 95 percent nitrogen, i.e., a reducing gas atmosphere. In batch annealing the strip is wound into a tight coil and subjected to the "box annealing" cycle, i.e., about ten hours at 1220°F., followed by a cooling cycle, all taking place under a protective gas atmosphere.

Following the annealing operation, the steel strip is usually stored to await further processing. It is during this storage period that rust formation is observed on steel strip that has not been treated with an inhibiting composition.

The good results of this invention are verified by a laboratory simulation of commercial steel strip manufacture and annealing. In these tests 3 inch × 6 inch panels (about 0.009 inch thick) of cold-rolled steel strip are electrocleaned in conventional alkaline silicate (sodium orthosilicate) cleaning solution. Half of the panels (the controls) are waterrinsed, and dried. The other half are dipped in an aqueous solution of one or more rust-preventing agents at various concentrations, and then dried. The various rinse compositions are summarized as follows:

| Test No. | Rinse Solution  |                 | Additives, Concentrations in g/liter |                        |                        |
|----------|-----------------|-----------------|--------------------------------------|------------------------|------------------------|
|          | Calcium Acetate | Calcium Nitrate | Sodium Nitrite                       | Potassium Ferricyanide | Potassium Ferrocyanide |
| 1        | 0               | 0               | 0                                    | 0                      | 7.5                    |
| 2        | 0               | 0               | 4.5                                  | 0                      | 0                      |
| 3        | 0               | 0               | 0                                    | 6.6                    | 0                      |
| 4        | 3.6             | 0               | 0                                    | 0                      | 0                      |
| 5        | 0               | 4.7             | 0                                    | 0                      | 0                      |
| 6        | 3.0             | 0               | 4.5                                  | 0                      | 0                      |
| 7        | 2.15            | 0               | 0                                    | 0                      | 5.35                   |
| 8        | 3.4             | 0               | 0                                    | 0                      | 4.15                   |

The panels are stacked, placed in an annealing chamber, and squeezed together by placing a  $\frac{1}{2}$  inch steel plate on top of the stack to simulate a tightly wound coil of strip steel as formed in a commercial plant. The annealing chamber containing the panel bundle is charged to an annealing furnace and subjected to the "T-1" batch-annealing cycle (essentially 10 hours at 1,185° to 1,230°F., requiring about three hours to reach said temperatures, and followed by about a 12-hour cooling cycle) under a protective gas atmosphere consisting of 5 percent hydrogen and 95 percent nitrogen.

Corrosion resistance of the panels is measured by sealing the panel for 15 minutes in contact with moisture-laden air over water at 130°F. The other side of the panel is at ambient room temperature (70°-75°F.). The rating of "good" indicates a 50% reduction in rust for the panel exposed to the high humidity compared to a control panel (blank) of the same metal similarly treated and exposed. In all cases the blank panels show a heavy blush of rust. A rating of "very good" indicates 75% reduction, and an "excellent" rating indicates a 90% or greater reduction in rust. The results are summarized as follows:

| Test No. | Rating and Appearance                           |
|----------|-------------------------------------------------|
| 1        | Very good; approximately 80% reduction in rust. |
| 2        | Good; approximately 50% reduction in rust.      |
| 3        | Good; approximately 75% reduction in rust.      |
| 4        | Good; approximately 65% reduction in rust.      |
| 5        | Fair; approximately 35% reduction in rust.      |
| 6        | Very good; approximately 75% reduction in rust. |
| 7        | Excellent; approximately 90% reduction in rust. |
| 8        | Very good; approximately 85% reduction in rust. |

I claim:

1. A process for inhibiting rust formation on cold-rolled steel strip which comprises contacting the strip, prior to annealing, with an aqueous dilute rinse solution containing an effective rust-inhibiting amount of a mixture of calcium ion and sodium nitrite, the calcium ion being supplied by a soluble calcium salt having a solubility in water of at least 1.88 g/liter of  $\text{Ca}^{++}$  ion and being free of corrosion-promoting anions selected from the class consisting of sulfate and chloride, wherein the concentration of calcium ion in the solution is from about 0.25 to 3 oz. per gallon and the concentration of sodium nitrite is from about 0.13 to 3 oz. per gallon, drying the steel strip and annealing the strip in a reducing gas atmosphere.

2. A process for inhibiting rust formation on cold-rolled steel strip which comprises contacting the strip, prior to annealing, with an aqueous dilute rinse solution containing an effective rust-inhibiting amount of a mixture of calcium ion and ferricyanide or ferrocyanide ion, the calcium ion being supplied by a soluble calcium salt having a solubility in water of at least 1.88 g/liter of  $\text{Ca}^{++}$  ion and being free of corrosion-promoting anions selected from the group consisting of sulfate and chloride, wherein the concentration of calcium ion in the solution is from about 0.25 to 3 oz. per gallon and the concentration of ferricyanide ion or ferrocyanide ion is from about 0.13 to 3 oz. per gallon, drying the steel strip and annealing the strip in a reducing gas atmosphere.

3. The process according to claim 1 wherein the calcium salt is selected from the group consisting of calcium acetate, calcium benzoate, calcium butyrate, calcium chromate, calcium ferrocyanide, calcium ferricyanide, calcium formate, calcium fumarate, calcium d-gluconate, calcium glycerophosphate, calcium isobutyrate, calcium iodide, calcium lactate, calcium  $\alpha$ -methylbutyrate, calcium nitrate, calcium nitrite, calcium propionate, calcium salicylate, calcium dithionate, calcium maleate and calcium valerate.

4. The process according to claim 2 wherein the calcium salt is selected from the group consisting of calcium acetate, calcium benzoate, calcium butyrate, calcium chromate, calcium ferrocyanide, calcium ferricy-

anide, calcium formate, calcium fumarate, calcium d-gluconate, calcium glycerophosphate, calcium isobutyrate, calcium iodide, calcium lactate, calcium  $\alpha$ -methylbutyrate, calcium nitrate, calcium nitrite, calcium propionate, calcium salicylate, calcium dithionate, calcium maleate and calcium valerate.

5. The process according to claim 4 wherein the ferricyanide or ferrocyanide ion is supplied by a salt se-

lected from the group consisting of ammonium ferricyanide, ammonium ferrocyanide, calcium ferricyanide, calcium ferrocyanide, magnesium ferrocyanide, potassium ferricyanide, potassium ferrocyanide, sodium ferricyanide, sodium ferrocyanide and strontium ferrocyanide.

\* \* \* \* \*